

# UNITED STATES PATENT OFFICE.

ADOLPH COHN, OF NEW YORK, N. Y.

## ALLOY.

1,323,833.

Specification of Letters Patent. Patented Dec. 2, 1919.

No Drawing.

Application filed May 2, 1919. Serial No. 294,183.

*To all whom it may concern:*

Be it known that I, ADOLPH COHN, a citizen of the United States, and a resident of the borough of Manhattan, city, county, and 5 State of New York, have invented certain new and useful Improvements in Alloys, of which the following is a specification.

This invention relates to a new alloy of precious metals and its object is to provide 10 a novel and comparatively inexpensive way of hardening platinum for the purpose of rendering it suitable for use in jewelry or for any other desired reason.

It is of course well known that pure platinum is too soft to resist wear and various 15 expedients have been resorted to with varying degrees of success, for the purpose of overcoming this difficulty.

I have discovered that the addition of a 20 very small proportion of gold has the desired hardening effect. A decided hardening of platinum is attained by the addition of as little as 1% of gold. It is my present belief that no more than 15% of gold in a 25 given amount of alloy is ever needed for this purpose. While I do not intend to limit myself in this particular, but as an exemplification of my invention, I have found by

scleroscope tests that an alloy of 95% platinum and 5% gold is equal in hardness to a 30 10% iridium-platinum alloy.

Another advantage of the use of gold as a 35 hardening agency for platinum is that these two metals alloy readily and form a perfectly homogeneous and permanent mixture. 40 These metals form an alloy which will not tarnish. They also form an alloy which is more easily soldered than is either pure platinum or iridio-platinum, and which has sufficient ductility to be wrought cold or hot, 45 and is also capable of being repeatedly melted without destroying its character.

I am aware of the fact that gold which has less than half of the hardness of platinum, has had its hardness increased by the 45 addition of a small percentage of platinum, but believe that it is new to increase the hardness of platinum by the addition of a comparatively small quantity of a softer metal such as gold. 50

What I claim is:

An alloy of platinum and gold with the gold from 1% to 15% of the whole.

In witness whereof I have hereunto set my hand this 1st day of May, 1919.

ADOLPH COHN.